

# United States Patent Office

2,873,203

Patented Feb. 10, 1959

1

2,873,203

## LIQUID ROSIN SIZES CONTAINING ANTI-STRATIFYING AGENT

William C. Hopkins, Valdosta, Ga., and John G. Senese, Jr., South Charleston, W. Va., assignors to American Cyanamid Company, New York, N. Y., a corporation of Maine

No Drawing. Application February 25, 1954  
Serial No. 412,636

5 Claims. (Cl. 106—238)

The present invention relates to rosin sizes. More particularly, the present invention relates to liquid rosin sizes containing a small but effective amount of sodium chloride as agent inhibiting stratification of these sizes on storage.

Rosin sizes have their principal use in the manufacture of paper. These sizes are manufactured on a large commercial scale by heating a natural or modified rosin above its melting point, forming a hot caustic solution from water and an alkali metal alkali such as potassium or, more commonly, sodium hydroxide or carbonate, and reacting the alkali solution with the rosin. The rosins referred to are organic acids. Neutralization of these acids by the caustic takes place within a few hours, the product being a viscous soap dispersion. In this process, the amount of water employed is controlled so that the size contains between about 50% and 80%—85% of size solids, on the one hand to avoid sizes so dilute that they cannot be shipped economically, and on the other hand to avoid sizes so concentrated and, therefore, viscous that they cannot be pumped.

The amount of alkali employed in this manufacture is at least about 60% of that required for complete neutralization so that the size contains up to about 40% of free rosin acids, based on the weight of the solids therein, a lower amount of alkali yielding a size which contains so much free rosin acids that it cannot be successfully diluted for application to paper. On the other hand, the amount of alkali may be sufficient to completely neutralize the rosin, and this yields satisfactory sizes.

In commercial practice, liquid rosin sizes generally contain between 60% and 80% of size solids by weight, thus minimizing shipping costs while providing a product having a pumpable viscosity at a temperature of about 60°—70° C., this being the standard temperature at which sizes are handled within paper mills. Moreover, sufficient alkali is used to cause at least 95%—75% neutralization of the rosin, this amount insuring that the rosin possesses excellent dilutability in water while maintaining consumption of alkali and the viscosity of the product at minimum practical values.

Frequently, liquid rosin sizes are stored by the manufacturer before they are shipped in tank cars, and these sizes are further stored by paper manufacturers before use. It is known that during these periods of storage liquid rosin sizes of the commercially practicable types mentioned, that is, sizes containing from about 5% to 25% of free rosin acids and about 60% to 80% of solids, stratify on storage and separate into two layers. The bottom layer is more viscous than the upper layer. Hence, when a liquid rosin size has been prepared of maximum pumpable viscosity, allowance being made for the increase in viscosity which normally takes place on aging, storage of the size results in separation of a bottom layer which is beyond the range of normal pumpability and which, therefore, can be removed from the storage tank only with difficulty.

A further disadvantage is that the upper layer is usually

2

darker in color than the lower layer, and this introduces a problem of color control in the manufacture of paper.

Stratification of liquid rosin size often becomes evident in the laboratory in 3—5 hours and, in the case of rosin stored in large commercial tanks, in about 3 days. The phenomenon is not spontaneously reversible and homogeneity can be obtained only by thorough mixing of the contents of the tank.

The discovery has now been made that liquid rosin sizes of the composition mentioned containing a small amount of sodium chloride do not stratify or otherwise separate on storage. The stratification is inhibited by the presence therein of between about 0.7% and 2% by weight of dissolved sodium chloride based on the weight of solids in the size and substantially completely inhibited by the presence therein of between about 2% and 5% by weight of dissolved sodium chloride based on the weight of solids in the size. It has further been found that separation of the sizes into phases takes place when more than about 5% of sodium chloride is present, the sodium chloride in this instance acting to "salt out" the rosin soap resulting also in an actual increase in viscosity of the size.

From the foregoing it will be seen that the subject matter of the present invention comprises a liquid rosin size of about 5% to 25% free rosin acids content containing about 60% to 80% size solids by weight, said size being inhibited against stratification on storage by the presence of an effective amount between about 0.7% and 5%, based on the weight of the solids, of sodium chloride dissolved therein, the amount of said sodium chloride being insufficient to salt out said size.

The amount of sodium chloride which should be present within the range mentioned varies with the type of rosin employed, the solids content of the size, the amount of free rosin acids in the size, and the temperature of the size. As a result, the minimum effective amount can best be determined in each instance by laboratory trial. In general, with regard to liquid rosin sizes of the composition mentioned, we have found that fortified rosin sizes of low solids content but containing an intermediate amount of free rosin acids show the greatest and most rapid stratification, and that with regard to these sizes, higher temperatures favor stratification. For example, a fortified rosin size containing 60% or 70% solids and 15% of free rosin acids is particularly prone to stratify and requires somewhat more sodium chloride for stabilization at the upper normal storage temperature of 80° C. than does ordinary rosin size containing 80% solids and 15% free rosin acids at the lower normal storage temperature of 50° C.

In place of sodium chloride, no reason is known why other alkali metal halides such as sodium bromide and sodium iodide as well as the corresponding potassium salts are not also effective, and these salts are therefore included within the broad scope of the present invention.

Because of its ready availability and the excellent results which it affords, sodium chloride is preferred, and in commercial practice common rock salt has proved entirely satisfactory.

In addition to inhibiting stratification it is a most important advantage of the present invention that the presence of sodium chloride very greatly decreases the viscosity of the sizes often to only a small fraction of the values which they would otherwise possess. Since the viscosity of liquid rosin sizes increases as their temperature falls, and since rosin sizes are normally stored in heated storage tanks, this means that rosin in such tanks can be stored at lower temperatures than would otherwise be the case. It is the customary practice of paper mills to store rosin size in tanks maintained at a temperature between about 60°—70° C. The presence of sodium

chloride permits the same sizes to be stored at a temperature about 20° C. lower without increase in viscosity, thus permitting substantial economy in the heat supplied.

It is a further advantage that the sodium chloride does not in any way alter the color of the size or affect the usefulness of the size in the manufacture of paper.

Freshly prepared liquid rosin size, when stored at normal temperatures within the range of 50°-80° C. increases rapidly in viscosity during the course of about the first seven days, the viscosity at that time often being several times that of the initial viscosity of the material. Thereafter the viscosity of the size generally remains at or near the high value reached towards the end of the first week of storage. It is a further most important advantage that the action of sodium chloride is a permanent one, the stabilized sizes of the present invention having a much lower viscosity during and after this period than corresponding sizes containing no sodium chloride.

In the manufacture of the liquid rosin sizes to which the present invention is directed, numerous forms of rosin are currently employed and include gum rosin, wood rosin, and tall oil rosin, the latter being a new development in the rosin field for which standards have been promulgated by the U. S. Department of Agriculture. Moreover, rosins may be employed which contain a minor amount, e. g. 10% to 40% by weight of the Diels-Alder adducts formed by reacting a naturally-occurring rosin with maleic anhydride or similar material. These rosins and the sizes prepared therefrom, generally respectively termed "fortified rosins" and "fortified rosin sizes" are disclosed broadly in U. S. Patents Nos. 2,628,918 and 2,385,794.

It will be understood that liquid rosin sizes, in addition to the foregoing, commonly contain a number of other materials. Included are the lower aliphatic alcohols and rosin esters therewith since rosin size may be prepared from rosin esters. Moreover, natural rosins contain small amounts of unsaponifiable materials including lignin and stearols. Sizes containing these materials undergo stratification on storage and the present invention is advantageously employed therewith.

The effect of sodium chloride in inhibiting stratification and decreasing the viscosity of a liquid fortified rosin size is illustrated as follows.

A liquid fortified rosin size was prepared by heating 15,000 pounds of M grade gum rosin to 150° C. and slowly adding 600 pounds of maleic anhydride. Reaction of the maleic anhydride was complete in 3 hours at about 170°-180° C., the product being fortified rosin containing the Diels-Alder rosin maleic anhydride product.

In a separate vessel 1,800 pounds of sodium hydroxide was dissolved in 23,700 pounds of water and the mixture heated to 95° C. The molten maleated rosin and the hot caustic solution were separately but simultaneously pumped into a cook tank and the mixture agitated by agitation of live steam from the bottom. Reaction of the caustic was complete in 2 hours. The resulting size had a free rosin acids content of 15% and a solids content of 70%.

Four samples, about a quart in size, were withdrawn. To one (Sample A) was added sufficient of a saturated aqueous sodium chloride solution to provide 0.7% of sodium chloride based on the weight of the solids therein. To the second (the control sample) was added an equal volume of deionized water. To the remaining samples were added saturated sodium chloride solution to provide sodium chloride in the amounts shown. All samples were stored at 80° C. and observed periodically for stratification. In addition, small amounts were removed periodically from the control sample and Sample A and their viscosity determined at the temperatures noted, the entire sample being first made homogeneous by stirring before the small amounts were withdrawn.

Stratification was deemed to take place when two distinct layers of different color could be observed. The samples were rated on an arbitrary scale on which 4 indicates bad stratification, 1 indicates acceptably slight stratification, and 0 indicates no noticeable stratification. Results are as follows:

| Sample      | Percent<br>NaCl <sup>1</sup> | Viscosity <sup>2</sup> at 55° C. |        |        |         | Viscosity <sup>2</sup> at 71° C. |        |        |         |
|-------------|------------------------------|----------------------------------|--------|--------|---------|----------------------------------|--------|--------|---------|
|             |                              | Start                            | 4 Days | 7 Days | 12 Days | Start                            | 4 Days | 7 Days | 12 Days |
| Cont'l..... | Nil                          | 17,700                           | 57,000 | 75,000 | 47,500  | 2,500                            | 9,500  | 11,500 | 8,400   |
| A.....      | 0.7                          | 5,000                            | 7,000  | 17,000 | 8,500   | 1,000                            | 1,200  | 1,800  | 1,500   |
| B.....      | 1.25                         | -----                            | -----  | -----  | -----   | -----                            | -----  | -----  | -----   |
| C.....      | 2.0                          | -----                            | -----  | -----  | -----   | -----                            | -----  | -----  | -----   |

<sup>1</sup> Based on solids content of size.

<sup>2</sup> Centipoises.

The sodium chloride may be introduced at any desirable point in the manufacture of the rosin size. For example, it may be dispersed into the molten rosin itself or may be dissolved in the liquid size subsequent to its preparation. Since, however, liquid rosin size is normally produced on a very large industrial scale it has been found most convenient to dissolve the sodium chloride in the water in which the alkali metal alkali is dissolved. In this manner uniform distribution of the anti-stratification agent is most readily effected, and separate metering of the agent becomes unnecessary.

In the present specification, the term "percent free rosin acids" is used to designate the proportion of the rosin acids, as found by titration, which are not neutralized by the alkali-metal alkali during manufacture of the size.

The invention will be more particularly described with reference to the examples which follow, which are intended only to illustrate specific embodiments of the invention and which are not to be construed as limitations thereon.

| Sample      | Stratification <sup>1</sup> |        |         |
|-------------|-----------------------------|--------|---------|
|             | 4 Days                      | 7 Days | 12 Days |
| Cont'l..... | 4                           | 4      | 4       |
| A.....      | 3                           | 3      | 3       |
| B.....      | 1+                          | 1+     | 1+      |
| C.....      | 0                           | 0      | 0       |

<sup>1</sup> On storage at 80° C.

65

These tests show that the presence of 0.7% and 1.25% of sodium chloride inhibits stratification and that increasing the amount to 2% substantially prevents stratification. The tests further show that only 0.7% of sodium chloride causes a sharp reduction in the viscosity of the size throughout the test. From previous experience it is known that the viscosity of rosin sizes containing 2%-5% of sodium chloride is less than the viscosity of similar sizes which contain 1.25% of sodium chloride.

**Example 2**

The effect of increasing amounts of sodium chloride upon the stratification of and viscosity of rosin size is illustrated by the following.

A fortified rosin size containing 72.5% solids and 9.6% free rosin was made by the method of Example 1, and a control sample and sodium chloride-containing samples were prepared also as described in Example 1. The initial viscosity of these samples was determined at 71° C. The samples were stored at 71° C. for two days and observed for stratification. Results are as follows, the stratification index being that of Example 1.

| Sample   | Percent NaCl <sup>1</sup> | Stratification at 2 Days | Viscosity at 71° C. (cp.) |
|----------|---------------------------|--------------------------|---------------------------|
| Control. | None                      | 4                        | 12,000                    |
| A        | 1                         | 4                        | 4,400                     |
| B        | 2                         | 1                        | 1,750                     |
| C        | 3                         | 0                        | 1,400                     |
| D        | 4                         | 0                        | 1,250                     |
| E        | 5                         | 0                        | 1,100                     |
| F        | 6                         | Salted Out               |                           |

<sup>1</sup> Based on the solids content of the size.

What is claimed is:

1. A liquid rosin size which is a uniform aqueous dispersion containing from about 60% to 80% rosin size solids by weight, and 5% to 25% of free rosin acids based on the weight of said solids, said size being inhibited against stratification on storage by the presence of an effective amount between 0.7% and 5%, based on the

weight of said solids, of sodium chloride dissolved therein, the amount of said sodium chloride being insufficient to salt out said size.

5 2. A liquid rosin size which is a uniform aqueous dispersion containing from about 60% to 80% rosin size solids by weight, and 5% to 25% of free rosin acids based on the weight of said solids, said size being stabilized against stratification on storage by the presence of an effective amount between 2% and 5%, based on the weight of said solids, of sodium chloride dissolved therein, the amount of said sodium chloride being insufficient to salt out said size.

10 3. A liquid maleated rosin size according to claim 2.

4. A liquid rosin size which is a uniform aqueous dispersion containing about 70% rosin size solids by weight, and about 15% free rosin acids based on the weight of said solids, said size being stabilized against stratification on storage by the presence of an effective amount between 2% and 5%, based on the weight of said solids, of sodium chloride dissolved therein, the amount of said sodium chloride being insufficient to salt out said size.

15 5. A liquid maleated rosin size according to claim 4.

**References Cited in the file of this patent****UNITED STATES PATENTS**

|              |         |                |
|--------------|---------|----------------|
| 83,707       | Gray    | Nov. 3, 1868   |
| 405,269      | Menzies | June 18, 1889  |
| 2,192,488    | Reilly  | Mar. 5, 1940   |
| 30 2,213,943 | Auer    | Sept. 10, 1940 |